

## UNITED STATES PATENT OFFICE

2,156,348

## COPPER-ZINC ALLOYS

Wolf Johannes Müller and Moritz Niessner,  
Vienna, Austria, assignors to Oesterreichische  
Dynamit Nobel Aktiengesellschaft, Vienna,  
Austria, a firm of Austria

No Drawing. Application June 29, 1935, Serial  
No. 29,102. In Austria July 21, 1934

3 Claims. (Cl. 75—155)

It is known that gamma-brass, that is to say copper zinc alloys with a copper content of about 31—40%, i. e. alloys which are characterised by a low copper content, are more resistant to corrosion than the brass alloys of the alpha and alpha and beta region with for instance 68—72% and more of copper, i. e. a higher copper content. The technical employment of gamma-alloys poor in copper is however impossible, since these alloys 10 are extremely hard and brittle and are consequently not machinable.

From such alloys as is described in our prior Patent Nos. 2,006,598 and 2,006,599, it has been disclosed that it is possible, by the addition of a few percent of a metal soluble in gamma-brass or alloyable therewith, such as nickel or, with more advantage cobalt, preferably by a simultaneous addition of nickel and cobalt, to obtain alloys, which possess the good resistance to corrosion of gamma-alloys poor in copper, but are also capable of being worked up, that is to say can be treated with machine tools and can also be rolled hot. Such alloys with an addition of approximately 3—10% of cobalt, nickel or the like 20 individually or in mixture, that is to say for instance pure copper-zinc alloys with a minimum content of nickel of approximately 7—8% or of cobalt of approximately 5—6% have extremely good technical properties, and when cobalt and nickel are used simultaneously it is possible with 25 a much smaller cobalt content to obtain the same effects as with the use of cobalt alone. Consequently alloys that are deficient in copper, even those most deficient, can be made utilisable for 30 industrial purposes or as constructional material for the production of articles, if the copper-zinc alloys are alloyed with cobalt, nickel or the like individually or in mixture.

The present invention is based on the discovery 40 that such copper-zinc alloys containing cobalt, nickel or the like, which contain copper in such an amount that they have a homogeneous mixed crystal or solid solution structure—that is to say in a binary system copper-zinc alloys with approximately 31—40% copper, can be substan-

tially improved in their properties by the addition of other metals, i. e. metals which are soluble in the solid solution of the alloy and are added or alloyed in an amount that is not greater than corresponds to their solubility in the solid solution. It has been found that such alloys can be made capable of being moulded in the cold state, i. e. rolled, pressed and drawn in the cold state by the addition of such metals in amounts which are soluble in the solid solutions so that the solid 10 solution formation is maintained and the occurrence of a heterogeneous structure is avoided. Such metals are for instance aluminium, tungsten, tin, chromium, selenium, tellurium, titanium, silver, silicon, iron, manganese, lead, molybdenum, zirconium etc. individually or two or more such metals combined as desired, and of these metals, the best effect is obtained by those which cause an increase in fineness of the grain, that is to say more especially manganese, iron, lead, 20 silver. Phosphorus also produces this effect. By such additions the region of the solid solution can also be somewhat extended with respect to that of the binary alloy, and alloys with a somewhat higher copper content for instance with 45% 25 copper content, which come in the beta and gamma region in the binary alloy, can be made suitable for purposes for which they would otherwise be impossible owing to their copper content, such as for instance for cold rolling or for a 30 drawing process.

In particular suitable are alloys with a copper content of at least 35%; such alloys, as compared with alloys with less copper content, have the advantage of better workability.

By addition of such metals the alloy can be improved in colour, more especially made whiter, and also favourably influenced as regards other properties, more especially made tougher, thus improving the capacity for being machined.

It is easily possible by empiric means to determine for each metal the amount which produces the most favourable effects.

It is more especially advisable to use the metals of the iron group, more particularly manganese,

5

15

20

25

30

35

40

45

which as compared with other metals, for instance as compared with aluminium, has the effect that with an increasing content, i. e. up to about 10%, there is an approximately proportional improvement in the capacity of working up cold, whereas for instance aluminium in amounts of about 0.3% has an extremely favourable action, but in amounts of more than 1.5% shows a diminished effect.

10 The more deficient the alloy is in copper, the greater addition of manganese is necessary, and the lower limit for alloys deficient in copper must be assumed as more than 4% manganese. The higher the content of manganese, the better is 15 the capacity for being worked up cold, and one can go up to an addition of about 15% manganese. Suitable is an alloy which beside manganese, contains iron up to the limit of solubility, which, depending on the composition of the alloy, may be 1 to 1.5%.

The addition of manganese has also the effect however that the addition of cobalt and nickel or the like can be reduced.

25 It is advisable to add very small amounts of phosphorus to such alloys, whereby a very considerable increase in the fineness of the grain of the alloys can be obtained.

The cobalt or nickel content or content of 30 cobalt and nickel in such alloys according to the invention may be between about 3-12%.

*Examples*

35 Suitable alloys according to the invention with manganese as added metal have for instance the following composition, it being clearly specified

however that the invention is naturally not limited to these examples:

|       | Percent by weight |
|-------|-------------------|
| 1. Cu | 37                |
| Ni    | 7                 |
| Co    | 2                 |
| Mn    | 7-8               |
| Zn    | Residue           |
| 2. Cu | 36                |
| Ni    | 6 10              |
| Co    | 2                 |
| Mn    | 10                |
| Fe    | 1.2               |
| Zn    | Residue           |
| 3. Cu | 45 15             |
| Ni    | 9                 |
| Co    | 1                 |
| Mn    | 8                 |
| Fe    | 1.0               |
| Zn    | Residue 20        |

What we claim is:

1. A corrosion resistant copper-zinc alloy, which is workable in the cold state, containing copper in an amount of 30 to 45%, at least one metal of the group cobalt and nickel in an amount of 3 to 12% and in addition thereto manganese in an amount 4 to 15%, the zinc constituting substantially the remainder. 25

2. An alloy according to claim 1 wherein the manganese content is smaller in the alloys of relatively high copper content than in the alloys of relatively low copper content. 30

3. An alloy according to claim 1 containing less than 40% copper.

WOLF JOHANNES MÜLLER.

MORITZ NIESSNER.

35